

May 10, 1966

H. HAYDN ET AL

3,250,616

PRINTING FORMS OF HIGH POLYMER SUBSTANCES

Filed Oct. 31, 1961



INVENTORS  
Hildegard Haydn  
& Edith Weyde

BY *Connolly and Kutz*  
ATTORNEYS

1

3,250,616

## PRINTING FORMS OF HIGH POLYMER SUBSTANCES

Hildegard Haydn and Edith Weyde, Leverkusen, Germany, assignors to Agfa Aktiengesellschaft, Leverkusen, Germany, a corporation of Germany

Filed Oct. 31, 1961, Ser. No. 148,844

Claims priority, application Germany, Nov. 16, 1960,  
A 36,944  
15 Claims. (Cl. 96—29)

This invention relates to printing forms of high polymer substances as well as to a process for the production of said forms by means of the silver salt diffusion process.

There are a number of well-known photographic processes of producing printing forms.

These methods include in particular the process of differentially hardening silver salt emulsion layers and transferring unhardened strata of such layers to a support to obtain useful printing forms. The binding agents of these layers are in general gelatin. It is also known, however, to replace the gelatin partially or completely by other polymeric substances or synthetic film-forming compounds that are capable of being tanned.

In this connection the silver salt diffusion process has already been used.

It is among the objects of the present invention to provide a novel method for producing printing forms by means of the silver salt diffusion process, whereby the differential hardening is obtained without the use of a hardening agent, thus providing printing forms with excellent physical properties. Other objects will be apparent from the following description.

We have found that film-forming polymeric natural or synthetic compounds containing carboxyl radicals or  $—COOX$  radicals in which X is a metal that are capable of reacting with silver ions to form polymeric silver salts serve as very useful binding agents for the transfer layers or printing matrix layers for the production of printing forms. By the formation of the silver salt the structure and the swelling properties of these polymeric compounds are changed in such a way that these areas become insoluble in water and have an imagewise differentiated adhesiveness of that high polymeric substance of the transfer layer to other materials.

According to a preferred embodiment of our invention, the adhesiveness of the transfer layer to the non-light-struck or unexposed areas of the negative silver halide emulsion layer can be improved by treating the negative layer with a solution containing development nuclei, preferably nuclei of metallic silver which are colloidally distributed therethrough or to add such nuclei or products that are capable of forming such nuclei on the surface of the negative to the developer solution. Thus it is possible to transfer these parts which have been entirely or partly converted into silver salt to another support by "tearing out."

High polymer substances having carboxyl groups which are particularly suitable for forming this layer include natural or processed natural products such as carboxymethyl cellulose, alginic acid and alginates and its derivatives and pectins. These compounds are chemically characterized in so far as they belong to the class of the carbohydrates having cyclic structures in particular of the pyranoside type substituted by a carboxyl grouping either directly at the ring or at a side chain. Thus the compounds contain approximately 10-50 percent, preferably 20-30 percent carboxyl groups per cyclic unit.

Carboxymethyl cellulose and processes for its preparation and structure are described by W. F. Waldeck and F. W. Smith, in Industrial and Engineering Chemistry, vol 44, pages 2803 to 2812 (December 1952), which was

2

reprinted in collaboration with Rodney N. Hader in "Modern Chemical Processes," which are volumes containing a series of articles describing chemical manufacturing plants by the editors of Industrial and Engineering Chemistry, III, pages 132 to 141, published by Reinhold Publishing Corporation, New York, 1954. Alginates or pectinic acid which are suitable for the process according to the invention are disclosed for example in "Recent Advances in Organic Chemistry" by Alfred W. Stewart and Hugh Graham, vol. II, pages 117-118, published by Longmans Green & Co., London, 7th ed., 1948 (Chapter IV, part B, entitled "Alginic Acid"), and in "Alginseide und Alginat" by H. Maas, SCT-Verlagsgesellschaft, Heidelberg, 1959, in particular pages 24 et seq., furthermore

15 "Chemische Textilfasern, Folien und Filme" by G. Pummerer, F. Enke Verlag, Stuttgart, 1953, pages 549 et seq.

Furthermore, synthetic resins containing carboxyl groups may be used, such as polymers of acrylic acid, maleic acid with a content of at least 20 percent of the acidic compound and similar substances that are capable of forming silver salts, furthermore, condensation products of formaldehyde with phenoxy acetic acid or other modified phenol formaldehyde resins containing carboxyl groups.

20 25 These polymeric products can be used in admixture with other film-forming polymers such as polyvinyl alcohols, gelatin, starch or starch derivatives and the like.

The transfer layer according to our invention may be prepared by casting a solution of the high polymer substance onto a paper carrier covered with hardened gelatin so that the polymeric substance does not penetrate into the paper support. The processes and printing forms of the present invention are described in the following general example:

30 35 A layer of carboxymethyl cellulose is cast onto a sheet of paper having a layer of hardened gelatin or other film-forming substance that produces a smooth surface. This transfer sheet consisting of the paper support and a transfer layer of carboxyl methyl cellulose is brought into contact with a negative silver halide emulsion layer that had been exposed to the object to be reproduced, after either layer has been moistened with a developer solution containing a solvent for silver halides. The light-struck areas of the negative are thereby reduced to silver while the silver halides of the non-light-struck areas are dissolved and transferred into the corresponding areas of the carboxymethyl cellulose layer, forming thereby polymeric silver salts and accordingly changing the chemical properties of these areas as described above, so that those areas

40 50 which correspond to the non-light-struck areas of the negative layer have a greater adhesiveness to the negative layer than to the underlying layer of hardened gelatin. If these two materials are now separated, the reacted portions of the carboxymethyl cellulose layer are present as a relief on the non-light-struck areas of the negative layer because the carboxymethyl cellulose layer at these areas has been torn out right down to the layer of hardened gelatin. At the same time, a relief is thereby formed on the carboxymethyl cellulose layer, wherein the depressions correspond to the original image. Both the relief formed on the negative layer and that remaining on the transfer layer may be used as a printing form.

55 60 65 The process of the present invention is also illustrated in and may be described by reference to the accompanying drawing, in FIG. 1 of which is represented a conventional light-sensitive negative sheet that consists of a support 1 to which adheres a layer of a light-sensitive silver-halide emulsion 2 and a separate transfer sheet that consists of a support 3 upon which is deposited a transfer layer 4 consisting of carboxymethylcellulose or

other suitable light-insensitive film-forming carboxy-substituted polymeric substances as described herein.

After being exposed to an image to be reproduced, the light-sensitive negative sheet is developed in a developer bath containing a silver-halide solvent. During or before the completion of the development, the transfer layer 4 of the transfer sheet is brought into contact with the wet silver-halide emulsion layer 2. During the development, a silver image is formed in the exposed areas 5 of the emulsion layer 2, as represented in FIG. 2, while the silver halide remaining in the unexposed areas of the emulsion layer 2 is dissolved by the silver halide solvent and diffuses into adjacent areas of the transfer layer 4 of the transfer sheet.

The developed negative sheet and the transfer sheet are then torn apart (separated) to produce two printing forms, which are represented in FIGS. 3 and 4, and are respectively a positive laterally reversed and a negative non-laterally reversed printing form. The areas of the transfer layer 4 which are adjacent the unexposed areas of the emulsion layer 2 (which are designated 6 in FIG. 3) adhere firmly to the emulsion layer 2 and are consequently torn out of the transfer layer 4 when the transfer sheet and negative sheet are torn apart.

The positive laterally reversed printing from that is thus obtained, which is represented in FIG. 3, consists of both the support 1 and emulsion layer 2 of the negative sheet and a relief layer consisting of the torn-out portions 6 of the transfer layer 4 of the transfer sheet.

The negative nonlaterally reversed printing form that is thus also obtained, which is represented in FIG. 4, consists of the support 3 of the transfer sheet and a relief layer consisting of the portions of the original transfer layer 4 (which are designated 7 in FIG. 4) that were adjacent to the exposed and developed areas 5 of the emulsion layer 2 and that were not torn out of the transfer layer 4 when the transfer sheet and negative sheet were torn apart.

From the negative nonlaterally reversed printing form represented in FIG. 4, a negative laterally reversed printing form can be made by bringing a sheet of tissue paper 8 into contact with the relief layer 7 of the printing form. FIGS. 5 and 6 show the relief layer 7 adhering to the sheet of tissue paper 8 producing on the tissue paper a negative laterally reversed relief layer that is suitable for use in spirit duplicating processes.

The positive laterally reversed printing form (FIG. 3) can be used in spirit duplicating processes to make prints by applying an alcohol-soluble dye to the relief layer. When an alcohol-soluble dye is incorporated originally in the transfer layer 4 of the transfer sheet, the relief layer of the resulting positive laterally reversed printing form can be used without further application of dye in the spirit duplicating process.

Relatively large quantities of other substances may be added to the transfer layer without substantially altering its properties. For example, considerable quantities of a dye may be incorporated into these layers. Thus by performing the process in accordance with the description herein of the invention, areas of the carboxymethyl cellulose layer corresponding to areas of the picture and containing relatively large quantities of a dye remain on the unexposed areas of the negative. In that case, a positive but laterally reversed picture of the original is produced on the negative. This negative may be used as a printing form for various processes depending on the type of dyes added. When using an alcohol-soluble dye in the layer, a larger number of copies can be obtained from the printing form of the negative using the process of spirit printing.

The relief remaining on the carboxymethyl cellulose layer may be used as a printing form for the template printing, for example, by transferring the layer which is still moist onto tissue paper. In that case, the pores of the tissue paper remain opened in those areas corresponding

to the picture, whereas in other areas they are occluded by the carboxymethyl cellulose layer. The printing dye or an alcohol-soluble dye can enter a paper carrier only through the open pores of the tissue paper. In that case again, one obtains a positive laterally non-reversed reproduction of the original.

As already mentioned above, a number of different coating agents may be used for the processes of the present invention which are characterized by containing carboxyl radicals that are capable of forming silver salts. A very large variety of substances may be used as additives. The choice of dye is determined by the printing process to be used.

Other additives which may be added to these layers influence mainly the swelling properties of the layer, which is important for the adhesiveness to the emulsion layer and to the underlying layer of hardened gelatin. For example, the addition of salts or of fillers which are not capable of swelling, such as barium sulphate, may have a profound effect on the behaviour of the transfer layer. The salt content of the developer or an addition of alcohol to the developer may also have a considerable influence on that layer. Principally it is possible to cast the layers directly onto a supporting sheet of paper. Preferably, however, the paper sheet should be coated with an intermediate layer of hardened gelatin, polyvinyl alcohol or other agents that produce a smooth surface. This is advantageous since the coating agent is prevented from diffusing or creeping into the material during the casting operation, which would make the subsequent transferring of portions of said layer more difficult. It is important that the transfer layers do not adhere too firmly to the support. Instead of paper, it has also been found satisfactory to use film foils in which case it is sometimes possible to omit the intermediate layer.

Experiments have shown that in each individual case the coating agent, support, and intermediate layer must be exactly adjusted to one another. This selection can be made without difficulties by those having ordinary skill in the art if the general description herein is followed.

As to the binding agent of the transfer layer it should be stated that by the term carboxy groups or radicals is to be understood in this connection free carboxyl groups as well as radicals having the formula  $-\text{COOX}$  in which X is a metal or other radical capable of neutralizing the carboxyl radical or replacing the hydrogen atom thereof. Both groupings are capable of reacting with silver ions to form the corresponding silver salts.

#### Example 1

|    |                                                                                                                                                                                                                                                                                                                                                                                                                                                                                                                                                                                                                |
|----|----------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|
| 50 | 1 liter of a 6.2 percent carboxymethyl cellulose (Phrikolat NV special containing about 40 percent salt) is intimately mixed with 30 grams Victoria Blue (Schultz, vol. 1, 7th edition, No. 822). After adding saponine, the solution is cast onto a paper which has previously been coated with polyvinyl alcohol. The layer produced is then treated, together with a photographic negative layer, preferably in an apparatus which is suitable for development in accordance with the silver salt diffusion process. The development may be performed with a developer which has the following composition: |
|    | Water, cc. ....                                                                                                                                                                                                                                                                                                                                                                                                                                                                                                                                                                                                |
|    | Sodium sulphite anhydrous, g. ....                                                                                                                                                                                                                                                                                                                                                                                                                                                                                                                                                                             |
|    | Sodium hydroxide anhydrous, g. ....                                                                                                                                                                                                                                                                                                                                                                                                                                                                                                                                                                            |
| 55 | Hydroquinone, g. ....                                                                                                                                                                                                                                                                                                                                                                                                                                                                                                                                                                                          |
|    | Phenidone (1-phenyl-3-pyrazolidone), g. ....                                                                                                                                                                                                                                                                                                                                                                                                                                                                                                                                                                   |
| 60 | Potassium bromide, g. ....                                                                                                                                                                                                                                                                                                                                                                                                                                                                                                                                                                                     |
|    | Sodium thiosulphate, g. ....                                                                                                                                                                                                                                                                                                                                                                                                                                                                                                                                                                                   |
|    | 1000                                                                                                                                                                                                                                                                                                                                                                                                                                                                                                                                                                                                           |
|    | 100                                                                                                                                                                                                                                                                                                                                                                                                                                                                                                                                                                                                            |
|    | 12                                                                                                                                                                                                                                                                                                                                                                                                                                                                                                                                                                                                             |
|    | 15                                                                                                                                                                                                                                                                                                                                                                                                                                                                                                                                                                                                             |
|    | 0.5                                                                                                                                                                                                                                                                                                                                                                                                                                                                                                                                                                                                            |
|    | 1                                                                                                                                                                                                                                                                                                                                                                                                                                                                                                                                                                                                              |
|    | 5                                                                                                                                                                                                                                                                                                                                                                                                                                                                                                                                                                                                              |

The exposed negative and the above-described carboxymethyl cellulose layer are together passed into the apparatus (through two separate slots) and the two layers are separated after about 2 minutes. After separation, the carboxymethyl cellulose dye layer remains only on the non-light-struck areas of the negative. The printing matrix

or form thus produced is suitable for spirit printing for which the usual printing apparatus may be used. 200 to 300 prints may be obtained from such a printing form.

The negative material was prepared as follows:

A sliver chloride-bromide gelatin emulsion is cast onto a paper support. An intermediate baryta layer may be recommendable in certain cases but is in general not necessary. The silver halide content of the light-sensitive layer, which may be additionally sensitized preferably to the blue and green region of the visible light amounts to 1.8-2.6 g. of silver per square metre. The layer is treated before or after being dried with a 0.5 percent dispersion of colloidally distributed metallic silver in water, thereby providing the surface of the light-sensitive emulsion layer with a small amount of silver nuclei.

*Example 2*

30 g. of Crystal Violet (Schultz, vol. 1, 7th edition, No. 785) are thoroughly mixed with 100 cc. of a 3 percent wax emulsion and dried. This dye-wax mixture is added to 1 liter of 5.4 percent carboxymethyl cellulose (Phrikolat NV special containing about 40 percent salts) on a paper which has been coated with hardened gelatin and it is then treated as described in Example 1.

*Example 3*

A 5 percent solution of carboxymethyl cellulose (Henkel G 5006), to which 10 percent of a non-swelling substance such as barium sulphate or titanium dioxide has been added as filler, is cast onto a paper which has a base layer of hardened gelatin. The layer is treated as described in Example 1. When the layer has been pulled off from the negative, it is placed while still wet onto a template of Japan paper or a fine fabric as generally used for wax stencil printing or screen printing. After drying for a short period, the layer adheres to the fibrous base. Since the portions of the carboxymethyl cellulose layer which correspond to the original image to be reproduced adhere to the negative, these parts are not transferred to the template. Thus the printing dye can penetrate through the pores of the material of the template.

*Example 4*

1 liter of Algipon 778 (of the firm Henkel) 0.9 percent, is mixed with 10 g. of Crystal Violet and 25 g. sodium chloride very thoroughly in a ball mill. The solution is cast onto paper which is covered with a hardened gelatin layer. The layers are treated as described in Example 1.

The present invention lends itself readily to a number of useful modifications in method, materials, apparatus, etc.

For example, the support of the transfer material may be paper with or without any immediate layer of a film-forming agent having a smooth surface, furthermore any film-forming polymer is suitable as a carrier, such as cellulose ester, polycarbonate, polyesters in particular those formed from terephthalic acid and ethylene glycol.

The printing dye may be incorporated into the transfer layer or may be applied in the form of a fatty printing ink to the final printing form. The chemical structure or the properties of the dye are not especially critical and are selected according to the requirements of the particular printing process in which the printing form is to be used. The same holds true with respect to the light-sensitive negative material which has no particular influence with respect to the process of the instant invention. It is only necessary that the portion of the transfer layer sufficiently adhere to the negative layer. This object is attained by treating the negative material with a solution or dispersion containing finely distributed particles of heavy metals such as silver, gold or the metals of subgroup VIII of the periodic system and metal sulfides or selenides such as cadmium selenide, silver sulfide or zinc sulfide. These nuclei operate in general as development nuclei and the improvement of the adhesion may prob-

ably be caused by a minor precipitation of sliver in the surface of said negative layer. The concentration of said nuclei necessary for obtaining the effect described above is very small, and is far less than the concentration of said nuclei in a commercial positive paper being used for the silver salt diffusion process, serving in this case for the precipitation of the silver halide which causes from the non-exposed and non-developed areas of the negative material and the formation of the positive image. Thus with the developing times being usual in the silver salt diffusion process no photographically disturbing silver precipitation is obtained at the non-light-struck areas of the negative material.

What is claimed is:

- 15 1. A process for simultaneously producing from a single negative (I) a positive laterally reversed printing form and (II) a negative non-laterally reversed printing form which comprises:
  - (a) exposing imagewise to an object to be reproduced a light-sensitive negative sheet comprising a light-sensitive silver halide layer adhering to a negative sheet supporting layer,
  - (b) developing the exposed light-sensitive negative sheet in a developer containing a silver halide solvent whereby the silver halide in the exposed areas of the emulsion layer is converted to a silver image and the silver halide in the non-exposed areas of the emulsion layer is dissolved,
  - (c) bringing the exposed emulsion layer of the negative sheet during development into contact with an amount of development nuclei sufficient to increase the adhesiveness of a transfer sheet to the emulsion layer but an amount less than that which causes a visible silver precipitation in the transfer sheet, said development nuclei being selected from the group consisting of heavy metals, heavy metal sulfides and heavy metal selenides and into contact with a transfer sheet, said transfer sheet consisting essentially of a transfer layer of a film-forming carboxy-substituted carbohydrate having a pyranoside structure and containing between 10 and 50 percent by weight carboxyl radicals adhering to a transfer sheet supporting layer whereby silver halide dissolved from the unexposed areas of the emulsion layer diffuses imagewise into the transfer layer thereby increasing imagewise the adhesiveness of the transfer layer to the emulsion layer, and
  - (d) separating the transfer sheet and the negative sheet whereby those portions of the transfer layer which were in contact with the unexposed areas of the emulsion layer now adhere to the emulsion layer and those portions of the transfer layer which were in contact with the exposed areas of the emulsion layer remain adhering to the transfer sheet supporting layer thereby producing (I) a positive laterally reversed printing form comprising the negative sheet and a relief layer of portions of the transfer layer and (II) a negative non-laterally reversed printing form comprising the transfer sheet supporting layer and a relief layer of the remaining portion of the transfer layer.
2. The process according to claim 1 wherein the development nuclei are selected from the group consisting of silver, gold, cadmium selenide, silver sulfide, zinc sulfide and metals of subgroup VIII of the Periodic System.
- 65 3. The process according to claim 1 wherein development nuclei are added to the developer prior to development.
- 70 4. The process according to claim 1 wherein the light-sensitive negative sheet is treated with a colloidal development nuclei dispersion.
- 75 5. The process according to claim 1 wherein the film-forming carboxy-substituted carbohydrate is selected from the group consisting of carboxymethylcellulose, pectins, alginic acid and salts of alginic acid.

6. The process according to claim 1 wherein the film-forming carboxy-substituted carbohydrate is carboxymethyl cellulose.

7. The process according to claim 1 wherein the film-forming carboxy-substituted carbohydrate is a salt of alginic acid.

8. The process according to claim 1 wherein the transfer layer contains an alcohol soluble dye.

9. A positive laterally reversed printing form comprising a printing form support sheet, a gelatin layer containing a silver image supported on said support sheet and a relief layer carried on and adhering to only those portions of the gelatin layer which contain no silver image, said relief layer comprising a film-forming carboxy-substituted carbohydrate having a pyranoside structure and containing between 10 and 50 percent by weight carboxyl radicals.

10. The printing form according to claim 9 wherein the relief layer is selected from the group consisting of carboxymethyl cellulose, pectins, alginic acid and salts of alginic acid.

11. The printing form according to claim 9 wherein the relief layer is carboxymethylcellulose.

12. The printing form according to claim 9 wherein the relief layer is a salt of alginic acid.

13. The printing form according to claim 9 wherein the relief layer contains an alcohol soluble dye.

14. A negative laterally reversed printing form comprising a printing form support sheet and relief layer

5 in the form of a negative non-laterally reversed image carried on said support sheet said relief layer comprising a film-forming carboxy-substituted carbohydrate having a pyranoside structure and containing between 10 and 50 percent by weight carboxyl radicals.

10 15. A negative laterally reversed printing form comprising a porous support sheet and a relief layer carried on said support sheet, said relief layer comprising a film-forming carboxy-substituted carbohydrate having a pyranoside structure and containing between 10 and 50 percent by weight carboxyl radicals.

#### References Cited by the Examiner

##### UNITED STATES PATENTS

|    |           |         |               |       |         |
|----|-----------|---------|---------------|-------|---------|
| 15 | 2,543,181 | 1/1951  | Land          | ----- | 96-29   |
|    | 2,923,623 | 1/1960  | Land          | ----- | 96-29   |
|    | 3,012,885 | 12/1961 | Abbott et al. | ----- | 96-35 X |
|    | 3,043,691 | 7/1962  | Weyde et al.  | ----- | 96-29   |

##### FOREIGN PATENTS

|         |         |                |
|---------|---------|----------------|
| 730,349 | 5/1955  | Great Britain. |
| 758,627 | 10/1956 | Great Britain. |
| 811,579 | 4/1959  | Great Britain. |
| 821,507 | 10/1959 | Great Britain. |

20 NORMAN G. TORCHIN, *Primary Examiner.*

LOUISE P. QUAST, *Examiner.*

A. D. RICCI, *Assistant Examiner.*